# EUROPEAN PATENT SPECIFICATION

(11) **EP 2 940 175 B1**
(45) Date of publication and mention of the grant of the patent: **03.02.2021**
(21) Application number: 13869412.0
(22) Date of filing: 19.12.2013
(51) Int. Cl.: C22C 38/00, C22C 38/58, C21D 8/00, C21D 6/00, C22C 38/06, C22C 38/34

(54) **DAMPING ALLOY**
DÄMPFUNGSLEGIERUNG
ALLIAGE AMORTISSEUR

(30) Priority: 28.12.2012 JP 2012287955
(43) Date of publication of application: 04.11.2015
(73) Proprietor: National Institute for Materials Science, Tsukuba-shi, Ibaraki 305-0047 (JP); Takenaka Corporation, Osaka-shi, Osaka 541-0053 (JP); Awaji Materia Co., Ltd., Hyogo 656-0015 (JP)
(72) Inventor: SAWAGUCHI Takahiro, Tsukuba-shi Ibaraki 305-0047 (JP); SAKURAYA Kazuyuki, Tsukuba-shi Ibaraki 305-0047 (JP); OGAWA Kazuyuki, Tsukuba-shi Ibaraki 305-0047 (JP); NAGASHIMA Nobuo, Tsukuba-shi Ibaraki 305-0047 (JP); FURUYA Yoshiyuki, Tsukuba-shi Ibaraki 305-0047 (JP); SEKIDO Nobuaki, Tsukuba-shi Ibaraki 305-0047 (JP); KOBAYASHI Satoru, Tsukuba-shi Ibaraki 305-0047 (JP); NAKAMURA Terumi, Tsukuba-shi Ibaraki 305-0047 (JP); NISHIMURA Toshiyasu, Tsukuba-shi Ibaraki 305-0047 (JP); TSUZAKI Kaneaki, Tsukuba-shi Ibaraki 305-0047 (JP); KUSHIBE Atsumichi, Inzai-shi Chiba 270-1395 (JP); INOUE Yasuhiko, Inzai-shi Chiba 270-1395 (JP); SUGATA Masahiro, Inzai-shi Chiba 270-1395 (JP); MARUYAMA Tadakatsu, Tokyo 101-0052 (JP); SUGIMURA Seiichi, Sumoto-shi Hyogo 656-0015 (JP); CHIBA Yuya, Tokyo 101-0052 (JP)
(74) Representative: Dehns
(86) International application number: PCT/JP2013/084119
(87) International publication number: WO 2014/103884

(56) References cited:
- CN-A- 1 399 002
- CN-A- 102 435 624
- JP-A- H1 036 943
- JP-A- S6 455 361
- JP-A- S62 112 751
- JP-A- S62 112 751
- JP-A- 2003 105 438
- JP-A- 2006 194 287
- SAWAGUCHI T ET AL: "Vibration mitigation by the reversible fcc/hcp martensitic transformation during cyclic tension-compression loading of an Fe-Mn-Si-based shape memory alloy", SCRIPTA MATERIALIA, ELSEVIER, AMSTERDAM, NL, vol. 54, no. 11, 15 March 2006 (2006-03-15), pages 1885-1890, XP027890448, ISSN: 1359-6462 [retrieved on 2006-06-01]

## Description

### Technical Field

The present invention relates to a damping alloy in which elasto-plastic deformation can be realized with low stress and fatigue properties are excellent.

### Background Art

Due to the Great East Japan Earthquake occurred on March 11, 2011 and the subsequent active seismic activity, disaster-prevention consciousness of great disaster is increasing in an unprecedented way. In particular, from the fact that areas where a strong earthquake is predicted include metropolitan areas, such as Tokai · Tonankai · Nankai earthquakes or an earthquake occurring directly beneath the Tokyo Metropolitan area, it has been made upmost efforts to reinforce and organize disaster prediction or disaster-prevention system and to also realize industrial disaster mitigation measures such as damping · seismic isolation techniques for preventing architectural constructions from earthquake damage.

A seismic damper is a seismic damping device which is configured to absorb vibration energy to be input to buildings by a wind or an earthquake such that the vibration does not reach a construction body. Seismic dampers which have been proposed and developed so far are roughly classified into a viscosity damper (see Patent Literature 1), a viscoelastic damper (see Patent Literature 2), a lead damper (see Patent Literature 3), an elasto-plastic damper (see Patent Literature 4), and the like.

Among these seismic dampers, the elasto-plastic damper using low-yield-point steel has recently become especially popular as a seismic damper for reducing the swing of the constructions at the time of the earthquake in particular due to excellence in performance, cost, and maintenance.

The elasto-plastic damper has a function of reducing the vibration of the building by mainly absorbing seismic energy to be input to the building as thermal energy due to plastic deformation of an alloy to be used as a core material for the damper.

Plastic deformation properties of the damping alloy as a core material have an important influence on the performance of the seismic damper. As for the plastic deformation properties of the damping alloy, to plastically deform earlier than construction body, yield stress or proof stress of the damping alloy is preferably low. In addition, since the core material itself for the damper is cyclically subjected to elasto-plastic deformation after the earthquake occurs, mechanical-property change or metal fatigue due to cyclic hardening is an issue from the viewpoint of long-term use.

The cyclic hardening is a cause of significant damage on a damping function of the seismic damper, for example, rising of operation start strength, and eventually even leads to destruction of the seismic damping device itself due to fatigue fracture when the metal fatigue proceeds. In order to avoid this situation, a damping alloy is expected in which a cyclic hardening rate is low and a fatigue life is long.

A damping alloy, which is most widely used now, is low-yield-point steel in which yield stress or 0.2% proof stress is intentionally reduced down to about 100 to 225 MPa; however, the damping alloy has a high initial cyclic hardening rate in the elasto-plastic deformation as the type of the yield stress is lower, and a fatigue life which is naturally superior to steel to be used in a main frame such as column and beam of constructions, but there is no significant difference in fatigue properties and it is hard to say that there is obvious superiority.

Accordingly, the conventional low-yield-point steel seismic damper has been inevitably designed in consideration of fatigue damage, for example, such that a core material is subjected to plasticity only at the time of the earthquake while not being subjected to plasticity (elastic range) at the time of swing by wind which is exposed to a large number of cycles at low strain amplitude (low amplitude).

In addition, after a big earthquake, it may be necessary to carry out inspection and replacement in some cases from a problem such as performance change or cumulative fatigue damage due to the cyclic hardening. Consequently, period and cost of disaster restoration occur.

Moreover, in recent years, attention has been paid to a problem of so-called long-period ground motion in which buildings such as skyscrapers resonate during the earthquake and thus swing of a relatively large deformation continues for a long period of time, and the request for a damping alloy having a longer fatigue life is increasing also from viewpoint of ensuring earthquake-proof safety of constructions.

Meanwhile, the fact that an Fe-Mn-Si-based shape memory alloy including NbC is available as a damping alloy of constructions, is disclosed by the inventors (for example, see Patent Literature 1).

This alloy is invented by giving attention to the fact that plastic strain remaining after the earthquake is removed by a shape memory effect due to heating and an initial shape can be restored. In addition, since a metallographic change of an alloy due to the tension-compression plastic deformation is reversibly carried out between a γ austenite phase of an FCC-type crystal (face-centered cubic lattice structure) and a ε martensite phase of an HCP-type crystal (hexagonal close-packed structure), other effects of the damping alloy has been also found that cyclic hardening rate is low and the fatigue life is also long (for example, see Non Patent Literature 1).

Typically, a mechanism for heating a damper member is required so as to utilize the shape memory effect; however, according to the proposal described above, even when the heating mechanism is not provided, it is possible to use it as a high-performance damping alloy which also effectively operates with respect to the long-period ground motion by the fact that the hardening rate due to at least a cyclic deformation is low and the fatigue life is long.

The fact that Fe-Mn-Si-based shape memory alloy is also effectively used as a damping alloy with almost same compositions is suggested in Patent Literature 5, but it also became obvious by the progress of subsequent research that the proper component range of the shape memory alloy did not fully match the proper component range of the damping alloy.

In Patent Literature 5, the alloy added with NbC to improve shape memory properties has extremely-high stress amplitude of 650 MPa or more with respect to cyclic tension-compression deformation at the amplitude of 1%. If the core material for the elasto-plastic damper is not subjected to elasto-plastic deformation earlier than the construction body, it is not possible to exhibit a vibration absorbing effect to protect the construction body.

That is, strength of the core material should be lower than that of the construction body of the building or the like. Accordingly, when a material having high material strength is used as the core material for the damper, it is necessary to make a cross-sectional area of the damper small so as not to exceed the strength of the constructions.

However, since a damper having a small cross-sectional area has a high buckling risk during the compression deformation, it is advantageous to lower the material strength of the core material for the damper to some extent to ensure a wide application range as a damper.

In order to solve this problem, the inventors attempted to control plastic deformation properties by making further investigation in such a manner that Al was added to an Fe-30Mn-6Si shape memory alloy as a base not containing precipitates such as NbC.

As a result, the fact is disclosed that an alloy containing Al of 1 to 3 mass% is effective as a damping alloy operable with low stress amplitude of about 300 MPa with respect to the cyclic tension-compression deformation at the amplitude of 1% (for example, see Patent Literature 6).

Meanwhile, according to Non Patent Literature 2, a shape memory effect almost disappears when Al exceeding 1 mass% is added to the Fe-30Mn-6Si shape memory alloy, and from this reason, it is also clear that the optimum component range of the shape memory alloy does not necessarily match that of the damping alloy.

In addition, it is an important request that the core material for the elasto-plastic damper can be produced at low costs using the existing mass steelmaking facilities to proceed earthquake resistance of the constructions promptly. Since the known damping alloy disclosed in Patent Literature 6 contains Mn of 30 mass% with a high concentration, it is difficult to make it using equipment such as an arc melting furnace in which common steel is produced.

The reason is that a boiling point of Mn is 2010°C which is very low compared to a boiling point 3070°C of Fe and oxides are easily produced by Mn rather than Fe, so that reduction in Mn yield due to evaporation or oxidation of Mn and reaction with refractories in the melting furnace inevitably occur, resulting in leading to difficulties even in terms of operation and cost. Therefore, from economical and technical requests, the development of an alloy having the lower content of Mn is essential to mass production and commercial viability of an Fe-Mn-Si-based damping alloy.

In the Fe-Mn-Si-based shape memory alloy, a component system is known in which some of Mn is substituted with Cr or Ni to improve corrosion resistance (for example, see Non Patent Literature 3); however, since this simultaneously cause the reduction of the content of Mn, it is suggested that the substitution with Cr or Ni is effective.

However, fatigue properties of the shape memory alloy obtained by substituting Mn with Cr or Ni are neither disclosed nor suggested so far. As described above, the proper component range of the shape memory alloy does not necessarily match that of the damping alloy. Accordingly, the optimum component range of the Fe-Mn-Cr-Ni-Si-based damping alloy is unclear. According to Non Patent Literature 4, secondary phases such as a δ ferrite phase, silicide, or an α' martensite phase are easily formed in the Fe-Mn-Si-based alloy added with Cr or Ni, but it is also unclear that these secondary phases have an influence on the fatigue properties.

Meanwhile, fatigue properties of an Fe-Mn-based austenitic steel are vigorously studied in recent years. This is because it has been recognized that twinning deformation of the γ austenite phase also has a good influence on the fatigue properties in TWIP (Twinning Induced Plasticity) steel to which attention is paid as a new automobile steel sheet excellent in strength ductility balance (for example, see Non Patent Literature 5).

Since the fatigue properties of the Fe-Mn-Cr-Ni-base alloy can be also examined from the same viewpoint, a relation between the fatigue properties and the structure has been partially known (for example, see Non Patent Literature 6). However, the plastic deformation structure of the Fe-Mn alloys or the Fe-Mn-Cr-Ni alloys is complex in which deformation twinning, the α' martensite phase, the ε martensite phase, stacking fault, dislocation, and the like are combined, and it is an indescribable situation that the relation between the fatigue properties and the structure is sufficiently elucidated.

From the experiment and research results so far by the inventors, it has been elucidated that the ε martensite is effective to the improvement of the fatigue properties, but it has not been almost elucidated that the ε martensite has the influence on the fatigue properties in the TWIP steel or the Fe-Mn-Cr-Ni-based alloy. Further, since the austenitic steel including the TWIP steel are designed as a typical structural material to have the components such that the yield strength is as high as possible, it is not suitable for the core material for the elasto-plastic damper.

As a damping alloy using the ε martensite phase, an Fe-Mn-Cr-Si-Al-C alloy is disclosed (for example, see Patent Literature 7). However, in the damping alloy, the γ austenite phase contains the ε martensite phase of 15% or more in a state before the deformation to improve internal friction in an elastic deformation region and the fatigue properties with respect to the elasto-plastic deformation are not disclosed.

The alloy has high strength because of previously containing the ε martensite phase in the state before the deformation or containing carbon which has the extremely strong nature of making solid-solution hardening of the γ austenite phase, and is not suitable for the core material for the elasto-plastic damper. Accordingly, components for increasing the fatigue life with the low proof stress and the low stress amplitude which are required for the damping alloy are neither disclosed nor suggested.

Patent literature 8 describes an Fe-Mn-Si shape memory alloy sheet metal.

As described above, the damping steel or the damping alloy, which are used for the main purpose of protecting the constructions from the earthquake as the core material for the elasto-plastic damper in the seismic damping device for the architectural constructions, requires the natures that the fatigue life is long (the number of cycles to fracture is large) with the low proof stress, the low cyclic hardening rate, and the large strain. However, the damping alloy having all of these natures in a good balance did not exist as the core material for the elasto-plastic damper. Patent Literature 9 describes a Fe-Mn-(Cr,Ni)-Si shape memory alloy having a high shape recovery.

### Citation List

### Patent Literature

Patent Literature 1: JP 5-263858 A
Patent Literature 2: JP 2001-146855 A
Patent Literature 3: JP 5-106367 A
Patent Literature 4: JP 5-26274 A
Patent Literature 5: JP 2006-194287 A
Patent Literature 6: JP 2008-56987 A
Patent Literature 7: JP 2011-214127 A
Patent Literature 8: JP S 62 112 751 A
Patent Literature 9: CN 1 399 002 A

### Non Patent Literature

Non Patent Literature 1: T. Sawaguchi, P. Sahu, T. Kikuchi, K. Ogawa, S. Kajiwara, A. Kushibe, M. Higashino, T. Ogawa, "Vibration mitigation by the reversible fcc/hcp martensitic transformation during cyclic tension-compression loading of an Fe-Mn-Si-based shape memory alloy" Scripta Materialia, 54 (2006) 1885
Non Patent Literature 2: M. Koyama, M. Murakami, K. Ogawa, T. Kikuchi, T. Sawaguchi, "Influence of Al on Shape Memory Effect and Twinning Induced Plasticity of Fe-Mn-Si-Al System Alloy" Mater. Trans. (2007)
Non Patent Literature 3: H. Otsuka, H. Yamada, T. Maruyama, H. Tanahashi, S. Matsuda, M. Murakami, "Effects of Alloying Additions on Fe-Mn-Si Shape Memory Alloys" Isij International, 30 (1990) 674
Non Patent Literature 4: B. C. Maji, M. Krishnan, V. V. R. Rao, "The microstructure of an Fe-Mn-Si-Cr-Ni stainless steel shape memory alloy" Met. Mat. Trans. A, 34A (2003) 1029
Non Patent Literature 5: T. Niendorf, F. Rubitschek, H. J. Maier, J. Niendorf, H. A. Richard, A. Frehn, "Fatigue crack growth-Microstructure relationships in a high-manganese austenite TWIP steel" Materials Science and Engineering a-Structural Materials Properties Microstructure and Processing, 527 (2010) 2412
Non Patent Literature 6: A. Glage, A. Weidner, H. Biermann, "Cyclic Deformation Behaviour of Three Austenite Cast CrMnNi TRIP/TWIP Steels with Various Ni Content" Steel Research International, 82 (2011) 1040

### Summary of Invention

### Technical Problem

The present invention aims to solve the conventional problems from the background as described above and an object thereof is to provide a damping alloy for an elasto-plastic damper such as an Fe-Mn-(Cr, Ni)-Si-based alloy in which proof stress and stress amplitude after cyclic tension-compression deformation are lowered and the number cycles to fracture is increased, the damping alloy being capable of being used in a maintenance-free manner even after long-period ground motion and being mass-produced.

### Solution to Problem

That is, the damping alloy of the present invention is characterized by claims 1 to 5.

### Advantageous Effects of Invention

Since the damping alloy of the present invention is configured such that the additive amount of Mn is set to be less than 20 mass%, it is also easily produced compared to the conventional Fe-30Mn-Si-Al-based damping alloy. In particular, the conventional Fe-30Mn-Si-Al-based damping alloy is melted only in a vacuum induction heating furnace, while there is a possibility of arc furnace melting when the additive amount of Mn is less than 20 mass% and thus a significant cost reduction is expected.

Furthermore, the damping alloy of the present invention has the number of cycles to fracture which is approximately one order of magnitude greater than that of the conventional low-yield-point steel for the elasto-plastic damper, and it can be also used against the long-period ground motion.

In addition, the damping alloy satisfying conditions defined in the present invention is configured in such a manner that the proof stress is 280 MPa or less, the stress amplitude is 400 MPa or less after the cyclic tension-compression deformation at the amplitude of 1% is carried out 100 times or more, and the number of cycles to fracture is 2000 cycles or more; and the damping alloy of the present invention is a damping alloy for an elasto-plastic damper which has the low proof stress or stress amplitude and can be operated at the low strength level, compared to the conventional Fe-Mn-Si-based shape memory and damping alloy including NbC, so that it can be applied to the damping member in a wide range.

### Brief Description of Drawings

Fig. 1 is a graph illustrating a relation between stress and strain of a first cycle of tension-compression deformation in Example 2 (4S).
Fig. 2 is a graph illustrating changes in stress amplitude by cyclic tension-compression deformation of alloys according to Examples and Comparative Examples.

### Description of Embodiments

Typically, a damping alloy indicates a structural material which absorbs mechanical vibrations in machine tools, precision equipment, automobiles, or the like by mainly realizing both of an increase of internal friction in an elastic deformation region and high strength as a metallic material.

In order to distinguish from this, meanwhile, the term "seismic damping" is sometimes used to describe damping for a main countermeasure against earthquake motion, but the term "damping" is being mainly used in recent years from the reason that control of ordinary vibration due to swing by wind other than the earthquake is also important to a damper for constructions.

According to this trend, the term "damping" is also used in the present invention, but the main subject thereof relates to vibration control on constructions during an earthquake. However, it is assumed that one of effects also includes the control of relatively small vibration due to the swing by wind or the like.

An damping alloy according to the present invention is an damping alloy in which elasto-plastic deformation reversibly takes place due to a mutual conversion of a γ austenite phase and a ε martensite phase by adjusting the content of Mn, Cr, Ni, and Si in an Fe-Mn-(Cr, Ni)-Si-based alloy and irreversible deformation such as a formation of an α' martensite phase is suppressed, such that proof stress is 280 MPa or less, stress amplitude is 400 MPa or less after cyclic tension-compression deformation at an amplitude of 1%, and the number of cycles to fracture is 2000 cycles or more.

In addition to slipping motion of lattice dislocations which is a plastic deformation mechanism of a general metal, a plastic deformation mechanism in an austenitic iron-based alloy takes various forms such as slipping motion of extended dislocations, in which a lattice dislocation is moved by being separated into two partial dislocations and a stacking fault sandwiched therebetween, twinning deformation, ε martensite transformation, and α' martensite transformation, and thus a plurality of plastic deformation mechanisms are usually expressed at the same time.

In the damping alloy according to the present invention, a structural change by tension-compression plastic deformation reversibly takes place due to two-directional martensite transformation between the γ austenite phase and the ε martensite phase, thereby suppressing cyclic hardening and increasing the number of cycles to fracture.

For this, a pre-deformation state is in a γ austenite single-phase, and the plastic deformation mechanism preferably proceeds mainly due to ε martensite transformation. At this time, twinning deformation, lattice dislocation slipping, or extension dislocation slipping, which occurs inevitably and concurrently with the ε martensite transformation, may be partially included, but α' martensite transformation should be suppressed because of significantly hardening an alloy.

Mn is an essential additive element having a critical influence on the plastic deformation mechanism of the Fe-Mn-(Cr, Ni)-Si-based alloy. Mn has a behavior of stabilizing the γ austenite phase and lowering stacking fault energy in the iron-based alloy, thereby easily occurring martensite transformation from the γ austenite phase to the ε martensite phase.

Accordingly, during the tension-compression plastic deformation, the ε martensitic transformation and reverse transformation thereof alternately occur from a deformation-induced γ, and the formation of the α' martensite phase can be suppressed, thereby improving fatigue properties.

Some of the austenite stabilizing function can be achieved using Ni instead of Mn, and some of the lowering function of the stacking fault energy can be achieved using Cr.

In order to reduce melting costs, the present invention necessarily includes Cr or Ni as an alternative additive element of Mn. Further, Al having an effect of improving the damping properties of an Fe-Mn-Si-based shape memory alloy may be also added as an alternative element of Mn.

An effect of Mn, Cr, Ni, or Al on the plastic deformation mechanism can be represented in terms of mass% of Mn having the same effect as those. In the present invention, this is defined as Mn equivalent weight ([%Mn]_{eq}), and the Mn equivalent weight is expressed by the following Formula (1) using the content (mass%) of each component element. $Mn equivalent weight \left({\left[%Mn\right]}_{eq}\right) = \left[%Mn\right] + \left[%Cr\right] + 2 \left[%Ni\right] + 5 \left[%Al\right]$

In the Formula, [%Mn], [%Cr], [%Ni], and [%Al] represent contents (mass%) of Mn, Cr, Ni, and Al as a chemical component of the damping alloy, respectively.

Furthermore, in the present invention the range of the Mn equivalent weight satisfies the condition expressed by the following Formula (2) to exhibit the two-way martensitic transformations between the γ austenite phase and the ε martensite phase. $37 < {\left[%Mn\right]}_{eq} < 45$

When the Mn equivalent weight is 37 mass% or less, the thermodynamic stability of the ε martensite phase becomes very higher, so that once the ε martensite phase is deformation-induced it will not be reversely transformed into the γ austenite phase even when it is deformed in a reverse direction.

As a result, the volume ratio of the ε martensite phase monotonously increases by the cyclic tension-compression deformation, and crack initiation probability or crack propagation rate rises at a place where the ε martensite phases, which have been formed, collide with each other and thus the number of cycles to fracture declines when the volume ratio is 50% or more by volume.

Furthermore, when the Mn equivalent weight is 30 mass% or less, since the ε martensite phase having the volume ratio of 15% or more by volume is already formed at the time of cooling from a solution heat-treatment temperature to a room temperature and a subsequent formation of a deformation-induced ε martensite phase is hindered, the number of cycles to fracture declines.

In addition, when the Mn equivalent weight is 45 mass% or more, the stacking fault energy increases and the ε martensite is not formed.

Meanwhile, Si as another essential additive element has little influence on the Mn equivalent weight, but it was apparent by experiments that Si improves reversibility of the two-directional martensite transformation between the γ austenite phase and the ε martensite phase and thus improves the number of cycles to fracture. Even when Si is not added, the number of cycles to fracture can be about 2000 cycles, but the number of cycles to fracture is more drastically increased by the addition of Si and the largest effect is exhibited when the additive amount of Si is near 4 mass%.

However, when Si is excessively added, the number of cycles to fracture is decreased, and, particularly, when Si is added to be 6.5 mass% or more, the alloy is significantly hardened, resulting in causing a problem that the stress amplitude of the cyclic tension-compression deformation rises in some cases.

In the additive amount of Mn, Cr, Ni, and Si, it is important to adjust the balance between the total amount of Ni and Mn which are austenite stabilizing elements and the total amount of Cr, Si, and Al which are ferrite stabilizing elements such that a metal structure before the deformation becomes a γ austenite single-phase. As the concentration of the ferrite stabilizing elements is high and the concentration of the austenite stabilizing elements is low, a δ ferrite phase is likely to form, and an α' martensite phase is likely to form when both of the concentration of the ferrite stabilizing elements and the concentration of the austenite stabilizing elements are low.

From experimental results by the inventors, when the alloy system of the present invention is water quenched after being subjected to a solution heat treatment at 1000°C for one hour, it has been found that the additive amount of component elements satisfied conditions of the following Formula (3) so as to suppress the formation of the δ ferrite phase and to make the γ austenite single-phase. $\left[%Ni\right] + 0.5 \left[%Mn\right] > 0.75 \left[%Cr\right] + 1.125 \left[%Si\right] + 2 [ %Al$

In the Formula, [%Ni], [%Mn], [%Cr], [%Si], and [%Al] represent contents (mass%) of Ni, Mn, Cr, Si, and Al as chemical components of the damping alloy, respectively.

The additive amount of each of Mn, Cr, Ni, Si, and Al as the component elements is limited by restrictions on production in addition to each condition described above. The description will be made below in detail.

### <Mn>

Mn is an essential additive element having two effects of austenite stabilization and stacking-fault energy reduction; in the damping alloy of Patent Literature 6 which is added with Mn of 30 mass%, however, reduction in Mn yield due to evaporation or oxidation of Mn and reaction with refractory in a melting furnace inevitably occur and it is difficult to melt at a practically allowable cost.

In the present invention, the additive amount of Mn is set to be less than 20 mass% by the addition of Cr or Ni to reduce the melting cost. Further, when the additive amount of Mn is less than 20 mass%, it is possible to produce an alloy using arc melting furnace which is suitable for mass production.

Meanwhile, when the additive amount of Mn is less than 10 mass%, both of Cr which is effective in the stacking-fault energy reduction and Ni which is the austenite stabilizing element should be added in great quantities, thereby causing the reduction in melting costs but allowing an increase in material costs.

Furthermore, when the additive amount of Mn is less than 5 mass%, the α' martensite phase harmful to the fatigue properties is inevitably formed even when the additive amount of Cr and Ni is adjusted in any way. From the above, in the present invention, the additive amount of Mn is preferably in the range of 5 mass% ≤ Mn < 20 mass%, and more preferably 10 mass% ≤ Mn < 20 mass%.

### <Cr>

Cr is an element which reduces the stacking-fault energy of the γ austenite phase and promotes the martensite transformation to the ε martensite phase, thereby improving the fatigue properties of the damping alloy according to the present invention. In addition, the element also contributes to improve corrosion resistance or high-temperature oxidation resistance. However, when the additive amount of Cr is 15 mass% or more, it is difficult to suppress the formation of the α' martensite phase even when the additive amount of other components is adjusted in any way and a low-melting point intermetallic compound is further formed by reacting with Si, so that it is difficult to melt the alloy. From the above, in the present invention, the additive amount of Cr is in the range of 0 mass% ≤ Cr ≤ 15 mass%.

### <Ni>

Ni is an alternative element of Mn for the austenite stabilizing behavior. In particular, when the additive amount of Mn is less than 20 mass%, the γ austenite single-phase, which is in a state before the deformation, is not obtained if Ni of 2 mass% or more is not added as an austenite stabilizing element.

Meanwhile, when the additive amount of Ni is 15 mass% or more, a low-melting point intermetallic compound is formed by reaction with Si, thereby deteriorating hot workability of an alloy.

In addition, from the viewpoint of material costs, the additive amount of Ni which is an expensive element is preferably less than 10 mass%. From the above, in the present invention, the additive amount of Ni is preferably in the range of 0 mass% ≤ Ni < 15 mass% and more preferably 2 mass% ≤ Ni ≤ 10 mass%.

With respect to Cr and Ni described above, at least either of both elements is contained in the damping alloy of the present invention and both elements are not set to be 0 mass% at the same time.

### <Si>

Si is an essential element of an Fe-Mn-Si-based shape memory alloy and the component range thereof is set to be 3.5 to 8 mass%, but the concentration of Si in a commercially available alloy is in the range of 5 to 6 mass% or less.

Meanwhile, even in the damping alloy of the present invention, Si is an element having an important role in improvement of the number of cycles to fracture, but the optimal component concentration therein is different from that in the shape memory alloy. From experiment and research results by the inventors, to obtain the number of cycles to fracture of 2000 cycles or more in the present invention, the additive amount of Si is in the range of 0 mass% < Si < 6.5 mass% and more preferably 2 mass% ≤ Si ≤ 6 mass%.

### <Al>

Al is an element having an influence on the Mn equivalent weight by factor 5 and thus may be added as an alternative element of Mn. However, since the element is also a ferrite stabilizing element, when Al is excessively added, the δ ferrite phase is easily formed. When a heat treatment is performed in an atmosphere, there is also a possibility that Al having high affinity with nitrogen forms nitrides to embrittle the alloy.

In this way, the Mn equivalent weight is effectively adjusted by adding even a trace amount of Al but a negative effect also occurs when Al is excessively added. Therefore, the additive amount of Al is in the range of 0 mass% ≤ Al < 3 mass%.

### <Others>

In the present invention, Co, Cu, C, or N may be added as an element having an alternative effect of Mn in addition to the above elements. However, since the addition of Co and Cu leads to an increase in material costs, the additive amounts of Co and Cu are in the following range in the present invention, respectively: Co < 0.2 mass% and Cu < 2 mass%.

In addition, since C and N cause a solid-solution hardening behavior of an alloy to increase yield strength and thus to impair performance of the alloy as a core material for an elasto-plastic damper, the upper limits of the additive amounts of C and N are in the following range, respectively: C < 0.1 mass% and N < 0.08 mass%.

In addition, for the purpose of removing interstitial elements C and N which are formed in an iron-based parent phase as a solid solution, carbides or nitrides are formed by the addition of an element such as Nb, Ta, V, Ti, or Mo having high affinity with C or N, which is widely carried out in the arts.

In the damping alloy of the present invention, it is necessary to minimize the effect of the solid-solution hardening of the parent phase due to the interstitial element C or N so as to reduce the proof stress or the stress amplitude in the cyclic tension-compression deformation. Therefore, even in the present invention, Nb, Ta, V, Ti, or Mo may be added by applying the conventional method so as to remove C or N formed as a solid solution.

However, when the additive amount of each element is too large, the proof stress or the stress amplitude increases on the contrary due to precipitation hardening of carbides or nitrides which are formed. In order to avoid this, each of the elements is in the following range in the present invention: Nb < 0.05 mass%, Ta < 0.05 mass%, V < 0.05 mass%, Ti < 0.05 mass%, and Mo < 0.05 mass%.

In the state before the deformation, the γ austenite single-phase is preferably formed, but the ε martensite phase may be formed in small quantity. In an alloy which is adjusted in a state where the ε martensite transformation is easily induced by the deformation, the ε martensite phase may be unintentionally formed in some cases due to an environmental temperature change, a machining influence or the like.

Since the unintentionally formed ε martensite phase differs from a subsequent deformation-induced ε martensite phase in a normal crystallographic orientation and becomes a barrier to the growth of the deformation-induced ε martensite phase, the volume ratio thereof is set to be less than 15 vol%.

The tension-compression plastic deformation of the damping alloy according to the present invention is mainly carried out in such a manner that the martensite transformation to the ε martensite phase from the γ austenite phase and the reverse transformation thereof alternately occur. The ε martensite phase induced at the time of the tensile deformation is reversely transformed to the γ austenite phase when a deformation direction is reversed to a compressive direction.

Meanwhile, the compressive deformation causes not only a reverse transformation of the tension-induced ε martensite phase but also a new ε martensite phase having a crystal orientation, which is different from a crystal orientation during the tension deformation. The compression-induced ε martensite phase is also reversely transformed to the γ austenite phase when the deformation is again reversed to the tension. In this way, since the increase in cumulative volume ratio of the ε martensite phase caused by the cyclic tension-compression deformation becomes smaller by cyclic formation and extinction of the tension-induced ε martensite phase and the compression-induced ε martensite phase in an alternate manner by the cyclic tension and compression, the damping alloy of the present invention has excellent fatigue properties.

However, the volume ratio of the ε martensite phase gradually increases as the strain amplitude or the number of cycles increases; and when the volume ratio thereof is 50% or more by volume, the crack initiation probability or the crack propagation rate increases, thereby causing the fracture in some cases. Accordingly, in order for that the number of cycles to fracture is 2000 cycles or more with respect to the tension-compression deformation at the amplitude of 1%, the volume ratio of the ε martensite is preferably less than 50 vol% after the deformation is carried out by the 2000 cycles.

In addition, since the α' martensite phase leads to hardening of the alloy, the volume ratio thereof should be less than 3 vol%. When the volume ratio of the α' martensite phase is 3% or more by volume, the stress amplitude increases due to the hardening; the increase in stress amplitude induces a new α' martensite phase transformation in a chain reaction, resulting in a decrease in the number of cycles to fracture as well as a decrease in damper performance due to an increase in stress level.

The proof stress of the damping alloy according to the present invention is set to be 280 MPa or less. When the proof stress is higher than this value, the cross-sectional area of the core material for the damper to be used to optimize the operation start strength of the damper becomes too small, the buckling easily occurs at the time of the elasto-plastic deformation. In order to avoid the buckling, a buckling stiffener should be provided, but the installation of the buckling stiffener leads to an increase in production costs of a damper member.

In addition, when the cyclic tension-compression deformation is carried out, the stress amplitude increases due to cyclic hardening, but from the viewpoint of long-term use, the stress amplitude is preferably set to be 400 MPa or less after the cyclic tension-compression deformation at the amplitude of 1 % is carried out 100 times or more.

When the stress amplitude exceeds 400 MPa, the yield strength of the core material for the damper rises to become higher than the strength of the building body after the big earthquake occurs, and thus it is difficult to operate as a damper in the subsequent earthquake. Since the damping alloy of the present invention is the core material for the seismic damper capable of corresponding even to the long-period ground motion and is intended to be used for the seismic damping device of a skyscraper, the final number of cycles leading to the fracture or buckling is 2000 cycles or more.

### Examples

The present invention will be described below in detail based on Examples. Naturally, the present invention is not limited by these Examples.

Each of alloys consisting of compound chemical compositions according to Examples 1 to 4 and Comparative Examples 1 to 8 indicated in Table 1 was prepared with 10 kg using a vacuum induction melting furnace, and after being subjected to hot forging and hot rolling at 1100°C, the prepared alloy was heated for one hour at 1000°C under an argon atmosphere and then was cooled with water thereby making an ingot. The additive amount of each component indicated in Table 1 is represented in terms of mass%.

In order to facilitate the understanding of features of compound components of Examples and Comparative Examples in Table 1, Examples 1 to 4 are also referred to as symbols 2S, 4S, 6S and 2A respectively and Comparative Examples 1 to 8 are also referred to as symbols 0S, 8S, 5M, 25M, 2N, 15N, PRE, and 30M1A, respectively.

**[Table 1]**

| | Symbol | Fe | Mn | Cr | Ni | Al | Si | Others | Mn equivalent weight |
|---|---|---|---|---|---|---|---|---|---|
| Example 1 | 2S | Bal. | 15 | 10 | 8 | 0 | 2 | | 41 |
| Example 2 | 4S | Bal. | 15 | 10 | 8 | 0 | 4 | | 41 |
| Example 3 | 6S | Bal. | 15 | 10 | 8 | 0 | 6 | | 41 |
| Example 4 | 2A | Bal. | 15 | 10 | 3 | 2 | 4 | | 41 |
| Comparative Example 1 | 0S | Bal. | 15 | 10 | 8 | 0 | 0 | | 41 |
| Comparative Example 2 | 8S | Bal. | 15 | 10 | 8 | 0 | 8 | | 41 |
| Comparative Example 3 | 5M | Bal. | 5 | 10 | 8 | 0 | 6 | | 31 |
| Comparative Example 4 | 25M | Bal. | 25 | 10 | 8 | 0 | 6 | | 51 |
| Comparative Example 5 | 2N | Bal. | 15 | 10 | 2 | 0 | 6 | | 29 |
| Comparative Example 6 | 15N | Bal. | 15 | 10 | 15 | 0 | 6 | | 55 |
| Comparative Example 7 | PRE | Bal. | 28 | 5 | 0 | 0 | 6 | 0.5vol%-NbC | 33 |
| Comparative Example 8 | 30M1A | Bal. | 30 | 0 | 0 | 1 | 5 | | 35 |

From each ingot of Examples 1 to 4 and Comparative Examples 1 to 8, a low-cycle fatigue test piece having a 8 mm-diameter parallel portion was prepared by lathe working and was subjected to a strain control low-cycle fatigue test at an amplitude of 1 % with a triangle wave of 0.1 Hz under an atmosphere of room temperature.

Fig. 1 illustrates a relation between stress and strain of a first cycle of tension-compression deformation in Example 2 (4S). From a state O with no deformation A, increase in tensile strain causes an elastic deformation OA, which is followed by a plastic deformation reaching to a point B, where tensile strain is 1%.

Thereafter, when the deformation is reversed to the compression, the curve reaches to a point D, where strain is zero, after an elastic deformation part BC in which tensile elastic stress decreases in proportion to a decrease in tensile strain as tensile plastic distortion gradually decreases.

When compression deformation further proceeds, compressive plastic strain occurs. When the compression strain reaches to a point E of -1%, the compression deformation is again changed into tensile strain, and an elastic deformation part EF is followed by a plastic deformation part FG to complete the first cycle. The second cycle starts along a curve GB' indicated by a dotted line, and then cyclic deformation is carried out in the same manner as the first cycle.

Work energy equal to an area drawn by the stress-strain curve formed in one-cycle deformation is converted into thermal energy, and is absorbed to mitigate the vibration.

During the tensile deformation, a start point of the plastic deformation was evaluated by 0.2% proof stress. In addition, a stress amplitude in the tension-compression deformation was obtained from tension-side maximum stress as illustrated in Fig. 1. The same evaluation was performed on all of the alloys according to Examples 1 to 4 and Comparative Examples 1 to 8. In addition, Fig. 2 illustrates changes in the stress amplitude by the cyclic tension-compression deformation of alloys according to Example 1 (2S), Example 2 (4S), Example 3 (6S), Comparative Example 1 (0S), Comparative Example 3 (5M), Comparative Example 4 (25M), Comparative Example 5 (2N), Comparative Example 7 (PRE), and Comparative Example 8 (30M1A).

Many alloys indicated a generally stable stress amplitude after being repeatedly hardened at initial 10 cycles. However, the alloy 5M was repeatedly hardened even after 10 cycles. In addition, the alloy PRE was initially hardened small and indicated a stable stress amplitude after being remarkably hardened from 10 cycles to 200 cycles. In order to evaluate the changes in the stress amplitude due to the cyclic tension-compression deformation, a stress amplitude (σa) at 100-th cycle was obtained and a hardening rate was calculated using the following Equation (4).$Hardening rate \left(H\right) = \left(σa100-σa1\right) / σ a 1$ Table 2 indicates proof stress, a stress amplitude at a first cycle, a stress amplitude at 100-th cycle, a hardening rate, and the number of final cycle obtained from these results.

**[Table 2]**

| | Symbol | Proof stress σ 0.2 (MPa) | Stress amplitude at first cycle σ a1 (MPa) | Stress amplitude at 100-th cycle σ a100 (MPa) | Hardening rate | Number of fracture cycles Nf (cycles) | Note |
|---|---|---|---|---|---|---|---|
| Example 1 | 2S | 201 | 230 | 364 | 0.58 | 3,222 | |
| Example 2 | 4S | 222 | 285 | 362 | 0.27 | 7,319 | |
| Example 3 | 6S | 260 | 333 | 400 | 0.20 | 4,506 | |
| Example 4 | 2A | 241 | 302 | 385 | 0.27 | 2,117 | |
| Comparative Example 1 | 0S | 160 | 201 | 337 | 0.68 | 1,992 | |
| Comparative Example 2 | 8S | - | - | - | - | - | Rolling crack |
| Comparative Example 3 | 5M | 256 | 298 | 572 | 0.92 | 282 | |
| Comparative Example 4 | 25M | 300 | 334 | 401 | 0.20 | 887 | |
| Comparative Example 5 | 2N | 248 | 401 | 671 | 0.67 | 474 | |
| Comparative Example 6 | 15N | - | - | - | - | - | Rolling crack |
| Comparative Example 7 | PRE | 290 | 495 | 620 | 0.25 | 3,002 | |
| Comparative Example 8 | 30M1A | 237 | 308 | 437 | 0.42 | 2,067 | |

In all alloys 2S, 4S, 6S and 2A according to Examples 1 to 4, the proof stress is 280 MPa or less, the stress amplitude at 100-th cycle is 400 MPa or less, and the final number of cycles is 2000 cycles or more. In the alloy 0S according to Comparative Example 1 not added with Si, the number of cycles to fracture was slightly below 2000.

In the alloy 8S according to Comparative Example 2 added with Si in larger amount than the component range of the present invention, it was not possible to prepare test pieces due to occurrence of rolling cracks. It was considered that the crack occurrence resulted from the formation of low-melting point intermetallic compounds.

In the alloy 5M according to Comparative Example 3 having the Mn equivalent weight less than 31, the cyclic hardening was significant and the number of cycles to fracture was also 1000 or less. It was considered that the cyclic hardening resulted from the deformation-induced α' martensite phase.

In the alloy 25M according to Comparative Example 4 having the increased Mn equivalent weight of 51, since the ε-phase is not formed by the deformation, the number of cycles to fracture was 1000 or less.

In the alloy 2N according to Comparative Example 5 in which the additive amount of Ni was 2 mass% lower than the inventive material and consequently, the Mn equivalent weight was reduced to 29, the cyclic hardening was significantly high and the number of cycles to fracture was also 1000 or less. It was considered that this resulted in the formation of the ε martensite phase of 50% or more by volume and the α' martensite phase.

In the alloy 15N according to Comparative Example 6 containing Ni of 15 mass% with more concentration than the alloys of Examples, cracks occurred during hot rolling, and thus test pieces could not be prepared. It was considered that this was because Ni formed a low-melting point intermetallic compound by reacting with Si.

The alloy PRE according to Comparative Example 7 is a damping alloy added with NbC precipitates which is disclosed in Patent Literature 5. The number of cycles to fracture is 3000 cycles or more which is excellent, but the stress amplitude is 620 MPa which is very high.

The alloy 30M1A according to Comparative Example 8 is an Al-added damping alloy disclosed in Patent Literature 6. The number of cycles to fracture is 2000 or more and the stress amplitude is also low, but since the content of Mn of 30 mass% is included, it is not suitable for mass production.

From these results, it was confirmed that the damping alloy according to Examples 1 to 4 satisfying conditions defined in the present invention is a damping alloy in which proof stress and stress amplitude after cyclic tension-compression deformation are lowered and the number of cycles to fracture is increased compared to the alloys according to Comparative Examples 1 to 8 deviated from the conditions of the present invention, the damping alloy being capable of being used in a maintenance-free manner even after long-period ground motion and being mass-produced.

### Industrial Applicability

By using the damping alloy according to the present invention, it is possible to manufacture a low-cost seismic damping device, which is capable of being operated at low stress and being used in maintenance-free manner even when being exposed to earthquakes repeatedly, as an elasto-plastic damper for restraining vibrations of architectural constructions caused by an earthquake, swing by wind, or the like.

As a high-performance damper without impairing the damping performance even when a large amplitude swing such as a long-period ground motion occurs for a long period of time, it is possible to be especially used in the damping of a skyscraper. In addition, it is expected that the effect of restraining the vibration of places deformed repeatedly by the large strain is exhibited in all forms of the architectural constructions such as chemical plants, power plants, halls, towers, fuel tanks, elevated railroads or roads, bridges, pipelines, tunnels, or wind power generation facilities.

## Claims

1. A damping alloy that is an Fe-Mn-(Cr, Ni)-Si-based damping alloy containing at least one of Cr or Ni, said damping alloy consisting of:
5 mass% ≤ Mn < 20 mass%;
0 mass% ≤ Cr ≤ 15 mass%;
0 mass% ≤ Ni < 15 mass%;
0 mass% < Si < 6.5 mass%; and
0 mass% ≤ Al < 3 mass%,
and optionally one or more of:
Co < 0.2 mass %;
Cu < 2 mass %;
C < 0.1 mass %;
N < 0.08 mass%;
Nb < 0.05 mass %;
Ta < 0.05 mass %;
V < 0.05 mass %;
Ti < 0.05 mass %, and
Mo < 0.05 mass %,
the balance being Fe and inevitable impurities, wherein
the component compositions satisfy the following conditions:
[%Ni] + 0.5 [%Mn] > 0.75 [%Cr] + 1.125 [%Si] + 2 [%AI]; and
37 < [%Mn] + [%Cr] + 2 [%Ni] + 5 [%AI] < 45, wherein [%Ni], [%Mn], [%Cr], [%Si], and [%AI] represent contents in mass% of Ni, Mn, Cr, Si, and Al, respectively.

2. A damping alloy as claimed in claim 1, wherein in said damping alloy Mn and Ni are present in the following amounts:
10 mass% ≤ Mn < 20 mass%; and
2 mass% ≤ Ni ≤ 10 mass%.

3. A damping alloy as claimed in claim 1 or claim 2, wherein in said damping alloy Si is present in an amount of 2 mass% ≤ Si ≤ 6 mass%.

4. A damping alloy as claimed in any one of claims 1 to 3, wherein
the metallographic structure of said alloy includes only a ε martensite phase, HCP structure, less than 15 vol% and a γ austenite phase, FCC structure, as a remaining part; and
when said alloy has been subjected to cyclic tension-compression deformation at an amplitude of 1% over 100 cycles or more, said alloy has a metallographic structure of the ε martensite phase less than 50 vol%, an α' martensite phase less than 3 vol%, and the γ austenite phase as a remaining part.

5. A damping alloy as claimed in any one of claims 1 to 4, wherein
proof stress is 280 MPa or less,
stress amplitude is 400 MPa or less after the cyclic tension-compression deformation at the amplitude of 1% is carried out 100 cycles or more, and
the number of cycles to fracture is 2000 cycles or more.

## Patentansprüche

1. Dämpfungslegierung, die eine Dämpfungslegierung auf Basis von Fe-Mn-(Cr, Ni)-Si ist, die Cr und/oder Ni enthält, wobei die Dämpfungslegierung aus Folgendem besteht:
5 Masse-% ≤ Mn < 20 Masse-%
0 Masse-% ≤ Cr ≤ 15 Masse-%
0 Masse-% ≤ Ni < 15 Masse-%
0 Masse-% < Si < 6,5 Masse-%; und
0 Masse-% ≤ Al < 3 Masse-%
und optional aus einem oder mehreren von:
Co < 0,2 Masse-%;
Cu < 2 Masse-%;
C < 0,1 Masse-%;
N < 0,08 Masse-%;
Nb < 0,05 Masse-%;
Ta < 0,05 Masse-%;
V < 0,05 Masse-%;
Ti < 0,05 Masse-% und
Mo < 0,05 Masse-%;
wobei der Rest Fe und unvermeidbare Verunreinigungen sind, wobei die Bestandteilzusammensetzungen folgende Bedingungen erfüllen:
[%Ni] + 0,5 [%Mn] > 0,75 [%Cr] + 1,125 [%Si] + 2 [%Al] und
37 < [%Mn] + [%Cr] + 2 [%Ni] +5 [%Al] < 45, wobei [%Ni], [%Mn], [%Cr], [%Si] und [%Al] für den Gehalt an Ni, Mn, Cr, Si beziehungsweise AI in Masse-% stehen.

2. Dämpfungslegierung nach Anspruch 1, wobei Mn und Ni in folgender Menge in der Dämpfungslegierung vorliegen:
10 Masse-% ≤ Mn < 20 Masse-% und
2 Masse-% ≤ Ni ≤ 10 Masse-%.

3. Dämpfungslegierung nach Anspruch 1 oder Anspruch 2, wobei Si in der Dämpfungslegierung in einer Menge von 2 Masse-% ≤ Si ≤ 6 Masse-% vorliegt.

4. Dämpfungslegierung nach einem der Ansprüche 1 bis 3, wobei
das Gefüge der Legierung ausschließlich eine ε-Phase Martensit, hdp-Struktur, von unter 15 Vol.-% und eine γ-Phase Austenit, kfz-Struktur, als übrigen Anteil beinhaltet; und
wenn die Legierung einer zyklischen Zug- und Druckverformung bei einer Amplitude von 1% über 100 oder mehr Zyklen ausgesetzt wird, die Legierung ein Gefüge aus der ε-Phase Martensit von unter 50 Vol.-%, einer α'-Phase Martensit von unter 3 Vol.-% und der y-Phase Austenit als übrigen Anteil aufweist.

5. Dämpfungslegierung nach einem der Ansprüche 1 bis 4, wobei
die Dehngrenze kleiner gleich 280 MPa beträgt,
die Spannungsamplitude kleiner gleich 400 MPa beträgt, nachdem die zyklische Zug- und Druckverformung bei der Amplitude von 1% über 100 oder mehr Zyklen durchgeführt wurde, und
die Zyklenzahl bis zum Bruch 2000 oder mehr Zyklen beträgt.

## Revendications

1. Alliage d'amortissement qui est un alliage d'amortissement à base de Fe-Mn-(Cr, Ni)-Si contenant au moins un de Cr ou Ni, ledit alliage d'amortissement consistant en :
5 % en masse ≤ Mn < 20 % en masse ;
0 % en masse ≤ Cr ≤ 15 % en masse ;
0 % en masse ≤ Ni < 15 % en masse ;
0 % en masse < Si < 6,5 % en masse ; et
0 % en masse ≤ Al < 3 % en masse,
et éventuellement un ou plusieurs de :
Co < 0,2 % en masse ;
Cu < 2 % en masse ;
C < 0,1 % en masse ;
N < 0,08 % en masse ;
Nb < 0,05 % en masse ;
Ta < 0,05 % en masse ;
V < 0,05 % en masse ;
Ti < 0,05 % en masse, et
Mo < 0,05 % en masse,
le reste étant du Fe et des impuretés inévitables, dans lequel
les compositions des composants satisfont aux conditions suivantes :
[%Ni] + 0,5 [%Mn] > 0,75 [%Cr] + 1,125 [%Si] + 2 [%Al] ; et
37 < [%Mn] + [%Cr] + 2 [%Ni] + 5 [%Al] < 45, dans lequel
[%Ni], [%Mn], [%Cr], [%Si] et [%Al] représentent les teneurs en % en masse respectivement de Ni, Mn, Cr, Si et Al.

2. Alliage d'amortissement selon la revendication 1, dans lequel dans ledit alliage d'amortissement Mn et Ni sont présents en des quantités suivantes :
10 % en masse ≤ Mn < 20 % en masse ; et
2 % en masse ≤ Ni ≤ 10 % en masse.

3. Alliage d'amortissement selon la revendication 1 ou la revendication 2, dans lequel dans ledit alliage d'amortissement Si est présent en une quantité de 2 % en masse ≤ Si ≤ 6 % en masse.

4. Alliage d'amortissement selon l'une quelconque des revendications 1 à 3, dans lequel
la structure métallographique dudit alliage inclut uniquement une phase de martensite ε, structure HCP, inférieure à 15 % en volume et une phase d'austénite γ, structure FCC, en tant que partie restante ; et
lorsque ledit alliage a été soumis à une déformation cyclique en traction-compression à une amplitude de 1 % sur 100 cycles ou plus, ledit alliage a une structure métallographique de la phase de martensite ε inférieure à 50 % en volume, d'une phase de martensite α' inférieure à 3 % en volume, et de la phase d'austénite γ en tant que partie restante.

5. Alliage d'amortissement selon l'une quelconque des revendications 1 à 4, dans lequel
la contrainte d'épreuve est de 280 MPa ou moins,
l'amplitude de contrainte est de 400 MPa ou moins après que la déformation cyclique en traction-compression à l'amplitude de 1 % a été effectuée 100 cycles ou plus, et
le nombre de cycles jusqu'à la fracture est de 2 000 cycles ou plus.
